

## UNITED STATES PATENT OFFICE

2,074,150

VAT DYE ASSISTANTS AND METHOD OF  
USINGJean G. Kern, Hamburg, N. Y., assignor to  
National Aniline and Chemical Company, Inc.,  
New York, N. Y., a corporation of New YorkNo Drawing. Application May 1, 1934, Serial  
No. 723,332

## 10 Claims. (Cl. 8—5)

This invention relates to the art of dyes and dyeing. It relates more particularly to a new class of vat assistants and to vat dye liquors or pastes and vat dyeing processes, especially printing pastes and printing processes comprising or employing such assistants, by means of which dyeings or prints of excellent fastness, depth, and brilliance may be obtained.

As is well known, vat dyes are water-insoluble solids and when used to dye textile fibers, they are ordinarily converted to a water-soluble (leuco) form (as by treatment with a reducing agent such as sodium hydrosulfite or formaldehyde sulfoxylate and potassium carbonate); in this form they are taken up by the fibers and are then rendered insoluble by an oxidizing or fixing treatment.

The printing process for dyeing textile fabrics generally involves applying a so-called printing paste to the fabric in the form of a design (for example by means of a screen, a stencil, or an engraved roll) and subsequently subjecting the printed fabric to further treatment to fix the dye upon the fibers.

Usually vat dye printing pastes contain, in addition to the vat dye, potential reducing agents,—substances which in themselves do not reduce the vat dye under the conditions of the printing operation but which upon application of heat with or without steam are capable of reducing the vat dye to the soluble leuco form. A mixture of sodium formaldehyde sulfoxylate and potassium carbonate is usually used as this reducing agent. The printing paste also ordinarily contains substances which promote the reduction of the dye or the absorption of the reduced compound by textile fibers, and suitable gums or thickeners. In some cases, as in printing with difficultly reducible vat dyes, the vat dye in the printing paste is subjected to a preliminary reduction before applying the printing paste to the fabric.

The heat treatment above referred to, ordinarily designated "aging", usually comprises subjecting the printed fabric to a short treatment with wet (saturated) steam while excluding oxygen, e. g., air, whereby the vat dye is reduced to the leuco form or its reduction is rendered more complete. This causes the dye to be absorbed more completely by the fiber.

After application of the printing paste to the fabric, and aging when this is employed, the fabric is subjected to an oxidizing treatment by passing it through an atmosphere containing

an oxidizing agent, e. g. air, or through a bath containing an oxidizing agent, e. g. a bath containing acetic acid and sodium dichromate. This oxidizing treatment converts the reduced vat dye compound back to the insoluble form upon the fiber. The fabric bearing the oxidized print is then washed, soaped, and rinsed, or otherwise suitably finished.

Vat dyes, when printed on textile fabrics with the aid of alkali-metal hydroxides, carbonates, or bicarbonates, frequently fail to yield full color value. This may be attributed to improper fixation of the dye on the fibers because of varying aging conditions or varying physical condition of the vat dye printing paste.

In accordance with the present invention, I have found that certain aryl ketones, though they themselves have no tinctorial power, nevertheless are excellent assistants or adjuvants for the application of vat dyestuffs in dyeing processes involving vat dyes. They are especially effective for assisting the conversion of vat dyes to their leuco form or for causing more complete conversion to this form, and hence they may be employed to advantage in all processes involving such a step. I have found, moreover, that vat dye printing pastes containing such compounds as assistants yield fast prints having excellent penetration, strength, and brilliance.

The ketones which I employ may be represented by the formula



wherein R represents an aryl radical of the benzene or naphthalene series, especially the former, and R' represents either a carboxyl group or a low-molecular alkyl, aryl, or aralkyl group, and wherein either R or R', or both, contain a group conferring solubility in water or alkaline solutions, for example an  $-SO_3Me$ ,  $-COOMe$ ,  $-OMe$ , or  $-SMe$  group, where Me represents hydrogen, a metal, an ammonium group, or an alkyl- or hydroxy-alkyl-substituted ammonium group (thus forming an amine salt). In view of their high water-solubility, I prefer to employ those ketones, the water-solubility conferring group of which is  $-COOMe$  or  $-SO_3Me$ , the latter especially. It will be understood that R and R' are separate radicals joined only through a single C=O group and that either or both may contain further substituents, e. g. alkyl-, oxy-, mercapto-, halogen-, sulfonate-, carboxy-, or amino-groups. As an example of amine salts

may be mentioned the amine salt of 2-benzoyl-benzoic acid and diethanolamine.

5



Examples of the aryl ketones suitable for the purposes of the present invention are the following acids or their salts, for example, their alkylamine and alkylolamine salts and their metal salts, especially their alkali-metal salts; e. g. those of Na and K:

15



20



25



30



35



40



45



50



55



60



65



70



75



The vat dye pastes of the present invention are suitable for application to the same types of fibers as ordinary vat printing pastes, for example, natural celluloses (e. g. cotton), regenerated celluloses, cellulose esters and ethers (e. g., the cellulose acetates and nitrates), and natural silk, as well as mixed goods manufactured from such fibers.

The printing pastes of this invention may be prepared in the usual manner with vat dyes of all types including those derived from anthraquinones, indophenols, various indigoid, thioindigoid and indirubin compounds, etc.; for example, indanthrones, pyranthrone, flavanthrones, dibenzanthrones, isodibenzanthrones, perylene quinones, anthanthrones, dibenzpyrene quinones, anthrimidocarbazols, naphthacridones, indigo, thioindigo, indirubin, etc. including derivatives thereof, such as their halogen, nitro, sulfur, and

alkoxy derivatives, either in reduced or unreduced form. The assistants described are especially satisfactory with dyes of the indigo and thioindigo series, however. The following dyes with which the invention may be employed to advantage are set forth to exemplify the general applicability of the invention:

|                                 | C. I. |
|---------------------------------|-------|
| Vat Orange R.                   | 1217  |
| 10 Tetrabrom Indigo             | 1184  |
| Indanthrene Blue GCD            | 1113  |
| Indanthrene Dark Blue BO        | 1099  |
| Flavanthrone                    | 1118  |
| Pyranthrone                     | 1096  |
| 15 Indanthrene Golden Orange R. | 1097  |
| Indanthrene Scarlet G.          | 1098  |
| Carbanthrene Blue Green FFB     | 1173  |
| Carbanthrene Violet 2R          | 1104  |
| Carbanthrene Red Violet 2RNX    | 1161  |
| 20 Carbanthrene Brilliant Green | 1101  |
| Vat Red Violet RH               | 1212  |
| Vat Scarlet G.                  | 1228  |
| Vat Pink FF (U. S. P. 892,897)  | 1222  |
| Vat Violet R.                   | 1222  |
| 25 Brilliant Indigo B.          | 1183  |
| Brilliant Indigo 4G             | 1189  |
| Dinaphthyl-thioindigo           |       |

The dye pastes or printing pastes of the present invention, of course, may contain the usual additions, among which may be mentioned alkaline reagents, e. g. alkali-metal hydroxides, carbonates, or bicarbonates, reducing agents, e. g., alkali-metal-hydrosulfites or alkali-metal-formaldehyde-sulfoxylates, and suitable thickening agents, e. g. starch, dextrin, mucilage, glue, British gum, gum arabic, and gum tragacanth. They may contain as well as the aryl ketones herein described assistants, such as glycerine, alcohols, ethers or amines, or hydrotropic reagents (as defined in my copending application Serial No. 673,031, filed May 26, 1933).

The application and development of printing pastes of the present invention may be effected in the customary manner for applying vat dye printing pastes.

The following examples will serve to illustrate the invention. Proportions are expressed as parts by weight.

Example 1.—1 part of sodium 2-benzoyl-benzoate is dissolved in 19 parts of a dyestuff paste containing 11.5% Vat Orange R (the remainder of the paste being mainly water, which may contain in addition a dispersing agent (leukanol) and/or glycerine). The resultant paste is intimately mixed with 80 parts of a reducing paste which is prepared by mixing 52 parts of a starch (British gum) tragacanth thickening paste [e. g. 2 parts cornstarch, 10 parts British gum, 2 parts 5% tragacanth (solution), and 38 parts water], 15 parts potassium carbonate, 16 parts water, 12 parts sodium formaldehyde-sulfoxylate, and 5 parts glycerine.

The printing paste so prepared is applied to textile fabric, e. g. a woven cotton fabric, in the usual manner.

The printed fabric is dried, exposed to air-free steam at about 102° C. for 3 to 5 minutes, and subsequently developed to yield a fast orange print by passing it through an aqueous bath which contains acetic acid and sodium dichromate and which is maintained at a temperature of 60° C. The developed print is then washed, soaped, rinsed, and dried in the usual manner. The orange print thus obtained has excellent penetra-

tion, is well-fixed to the fiber, and is ordinarily 15% to 20% stronger and more brilliant than prints obtained by the same procedure, omitting the sodium 2-benzoyl-benzoate from the printing paste.

Example 2.—1 part of the disodium salt of benzophenone-2-carboxy-4'-sulfonate is dissolved in 19 parts of a dyestuff paste containing 20% tetrabromindigo (the remainder of the paste being inert material). The resultant paste is intimately mixed with 80 parts of a reducing paste prepared as described in Example 1. This printing paste, upon application to and development upon a textile fabric, for example a cotton fabric, yields prints of superior brilliance and increased strength over those obtained with a printing paste lacking the disodium benzophenone-2-carboxy-4'-sulfonate but otherwise the same.

Example 3.—200 parts of a dyestuff paste containing 16% Indanthrene Blue GCD (C. I. 1113) are intimately mixed with 50 parts of the disodium salt of benzophenone-2-carboxy-4'-sulfonate, 3 parts sodium isopropylnaphthalene-sulfonate, and 115 parts of soluble dextrin. The homogeneous mixture thus obtained is dried in vacuum and ground to the desired fineness. The resultant powder can be used in the same manner as ordinary vat dyestuff powders for the production of prints on textiles and, when so applied, yields prints of high brilliance and strength.

Example 4.—10 parts of sodium isatinate are mixed with 120 parts of an aqueous Vat Pink FF paste containing 15% actual dye solids. The mixture is evaporated down to 100 parts. This mixture is then mixed with 400 parts of the reducing paste described in Example 1. The paste thus formed may be printed on cotton or other textile fabric, aged, and developed by the method of Example 1 yielding a fuller and stronger print than obtainable with omission of the sodium isatinate.

It is not necessary that the ketone be introduced as such into the paste but it may be formed from another compound or other compounds under the conditions of application and it will be understood that the invention includes such formation of the ketone within its scope. Thus, isatin, which when heated in alkaline media forms a salt of 2-amino-benzoyl-formic acid (isatinic acid), may be employed instead of the sodium isatinate of Example 4, as in the following example.

Example 5.—1 part of isatin is mixed with 19 parts of an aqueous 15% Vat Pink FF paste. The mixture is evaporated down to 19 parts. The mixture is then mixed with 76 parts of the reducing paste described in Example 1. The paste thus formed may be printed on cotton, aged, and developed by the method of Example 1. A fuller and stronger print is obtained than when the isatin is omitted. Since vat dye prints are aged by application of heat to the alkaline paste isatin present is converted to an alkali-metal isatinate. Accordingly either isatin or isatinic acid or a soluble isatinate may be used with substantially the same results.

It will be understood that the vat dye powders obtained according to the foregoing examples and/or other similarly obtained vat dye preparations, either in a paste or powder form, and containing the aryl-ketonic bodies as disclosed in this invention, may also be used for the tinting and dyeing of textile fibers by the methods referred to as dyeing operations, including as such the pad-jigg dyeing method, package dyeing

padding in a reduced vat dye bath, whereby excellent results are obtained. They may also be used for the production of white and/or colored discharge prints.

5 I claim:

1. In the preparation of dyed textile fibers, the step which comprises bringing the fibers into contact with a vat dyestuff and a non-foaming aryl ketone having the general formula



wherein R represents an aryl radical of the benzene or naphthalene series and R' represents a carboxyl group or a low molecular alkyl, aryl, or 15 aralkyl group, and which ketone contains a group conferring solubility in water or alkaline solution.

2. In the preparation of dyed textile fibers, the step which comprises subjecting a vat dyestuff in contact with the fibers to the action of a reducing agent in the presence of a non-foaming aryl 20 ketone having the general formula



wherein R represents an aryl radical of the benzene or naphthalene series and R' represents a carboxyl group or a low molecular alkyl, aryl, or aralkyl group, and which ketone contains a group conferring solubility in water or alkaline solution.

3. In the printing of a textile fabric, the step 30 which comprises applying to the fabric a printing paste comprising a vat dyestuff and a non-foaming aryl ketone having the general formula



35 wherein R represents an aryl radical of the benzene or naphthalene series and R' represents a carboxyl group or a low molecular alkyl, aryl, or aralkyl group, and which ketone contains a group conferring solubility in water or alkaline solution.

40 4. The method of producing a printed textile fabric, which comprises printing upon the fabric an alkaline paste comprising a vat dyestuff, a potential reducing agent, and a non-foaming aryl ketone having the general formula



wherein R represents an aryl radical of the benzene or naphthalene series and R' represents a carboxyl group or a low molecular alkyl, aryl, or 50 aralkyl group, and which ketone comprises a  $-COOMe$  or  $-SO_3Me$  group, Me representing an alkali-metal, and subsequently aging and developing the print.

5. A dyestuff composition comprising a vat 55 dyestuff and a non-foaming aryl ketone having the general formula



wherein R represents an aryl radical of the benzene or naphthalene series and R' represents a carboxyl group or a low molecular alkyl, aryl, or aralkyl group, and which ketone contains a group conferring solubility in water or alkaline solution.

6. A vat dye printing paste comprising a vat dye-stuff, a potential reducing agent, and an assistant, dispersed in an alkaline aqueous medium, said assistant comprising a non-foaming aryl ketone having the general formula



wherein R represents an aryl radical of the benzene or naphthalene series and R' represents a carboxyl group or a low molecular alkyl, aryl, or aralkyl group, and which ketone comprises a  $-COOMe$  or  $-SO_3Me$  group, Me representing an alkali-metal.

7. A vat dye powder comprising a vat dyestuff and a solid non-foaming aryl ketone having the general formula



wherein R represents an aryl radical of the benzene or naphthalene series and R' represents a carboxyl group or a low molecular alkyl, aryl, or aralkyl group, and which ketone contains a group conferring solubility in water or alkaline solution.

8. In the application of a vat dyestuff to textile fibers, the step which comprises subjecting fibers with the vat dyestuff thereon to an aging treatment in the presence of a non-foaming aryl ketone having the general formula



wherein R represents an aryl radical of the benzene or naphthalene series and R' represents a carboxyl group or a low molecular alkyl, aryl, or aralkyl group, and which ketone comprises a  $-COOMe$  or  $-SO_3Me$  group, Me representing an alkali-metal.

9. In the application of a vat dyestuff to textile fibers, the step which comprises bringing the fibers into contact with the vat dyestuff and an aryl ketone having the general formula



wherein R and R' represent aryl radicals of the benzene series, and which ketone comprises an  $-SO_3Me$  group wherein Me represents hydrogen or a metal.

10. In the preparation of dyed textile fibers, the step which comprises bringing the fibers into contact with a vat dyestuff and a diaryl ketone containing a group conferring solubility in water or alkaline solution.

JEAN G. KERN.